

# UNITED STATES PATENT OFFICE.

LEWIS D. SHIVLEY, OF KOKOMO, INDIANA.

## COMPOUND.

1,344,658.

Specification of Letters Patent. Patented June 29, 1920.

No Drawing.

Application filed October 16, 1919. Serial No. 331,126.

To all whom it may concern:

Be it known that I, Lewis D. SHIVLEY, a citizen of the United States, residing at Kokomo, in the county of Howard and State of Indiana, have invented a new and useful Compound, of which the following is a specification.

This invention relates to a composition with matter for use in tempering high speed steel in water and to the process of tempering the metal.

One of the objects of the invention is to provide a composition of this character which is inexpensive and which, when sprinkled on steel heated to the high temperature and subsequently dipped in water, will render the steel very hard and tough so as to be especially useful as a high-grade tool steel.

With the foregoing and other objects in view which will appear as the description proceeds the invention consists of the following ingredients substantially in the proportions stated:

|    |                            |        |
|----|----------------------------|--------|
| 25 | Soda ash                   | 2 lbs. |
|    | Borax                      | 1 "    |
|    | Boracic acid               | 1/2 "  |
|    | Sal ammoniac               | 2 oz.  |
|    | Salt peter                 | 1 "    |
| 30 | Magnesia                   | 2 "    |
|    | Yellow prussiate of potash | 1/2 "  |
|    | Potassium cyanid           | 1/4 "  |
|    | Manganese                  | 2 "    |
| 35 | Sulfur                     | 1/4 "  |
|    | Red lead                   | 5 "    |

The foregoing ingredients, with the exception of the soda ash, are thoroughly mixed, dried, and reduced to a powder, after which the composition is ready for use. To five gallons of water are added the two pounds of soda ash. The steel to be treated is heated approximately to 1500 degrees F. On this heated steel the powdered preparation is thoroughly sprinkled after which the metal is re-heated to approximately 2250 degrees F. This highly heated metal is then dipped in the mixture of water and soda

ash and it will be found, on removing the steel from the bath, that it has been tempered or hardened so as to constitute a high-grade tool steel.

In partial explanation of the foregoing operation it might be stated that after the metal has been heated the first time the composition is sprinkled on it and melts so as to form a coating. When the metal is again heated with this coating on it some of the ingredients of the coating impregnate the metal. It has been found that some chemical reaction upon the high speed metal takes place, but the exact nature of this re-action has not as yet been definitely determined. It has been proven by test, however, that steel hardened by the use of the composition such as herein described will stand up under greater heat and will take up and dispose of more heat while in use, than metal hardened by any other known process.

What is claimed is:—

1. A composition of matter for use in tempering steel including the following ingredients substantially in the proportion stated, soda ash 2 lbs., borax 1 lb., boracic acid  $\frac{1}{2}$  lb., sal ammoniac 2 oz., salt peter 1 oz., magnesia 2 oz., yellow prussiate of potash  $\frac{1}{2}$  oz., potassium cyanid  $\frac{1}{4}$  oz., manganese 2 oz., sulfur  $\frac{1}{4}$  oz., red lead 5 oz., and water 5 gallons.

2. The herein described method of tempering steel which consists in heating steel to approximately 1500 degrees F., sprinkling upon the hot steel borax, boracic acid, sal ammoniac, salt peter, magnesia, yellow prussiate of potash, potassium cyanid, manganese, sulfur, and red lead, re-heating the metal to approximately 2250 degrees F., and then immersing the metal in a bath consisting of 5 gallons of water and 2 pounds of soda ash.

In testimony that I claim the foregoing as my own, I have hereto affixed my signature in the presence of two witnesses.

LEWIS D. SHIVLEY.

Witnesses:

LESLIE O. MCVEY,  
CHAS. JINKERSON.